

# United States Patent [19]

Gauger et al.

[11] Patent Number: 4,459,324

[45] Date of Patent: Jul. 10, 1984

[54] ELECTRODE COATING WITH PLATINUM-GROUP METAL CATALYST AND SEMI-CONDUCTING POLYMER

[75] Inventors: Jürgen Gauger, Thonex; Jean-Marcel Hinden, Chambésy; Michael Katz, Geneva, all of Switzerland

[73] Assignee: Diamond Shamrock Corporation, Dallas, Tex.

[21] Appl. No.: 366,737

[22] Filed: Apr. 8, 1982

## Related U.S. Application Data

[63] Continuation-in-part of Ser. No. 282,182, May 21, 1981, Pat. No. 4,402,996.

## Foreign Application Priority Data

Apr. 9, 1981 [GB] United Kingdom ..... 8111258

[51] Int. Cl. <sup>3</sup> ..... B05D 5/12

[52] U.S. Cl. ..... 427/86; 427/125; 427/126.3; 427/126.5; 427/226; 427/388.2; 204/290 R

[58] Field of Search ..... 252/425.3; 427/126.5, 427/125, 126.3, 86, 87, 226, 388.2

## [56] References Cited

### U.S. PATENT DOCUMENTS

|            |         |                         |             |
|------------|---------|-------------------------|-------------|
| Re. 29,419 | 9/1977  | DeCraene .....          | 427/126.5 X |
| 3,632,498  | 1/1972  | Beer .....              | 204/290 F   |
| 3,881,957  | 5/1975  | Hausler .....           | 429/30      |
| 4,118,294  | 10/1978 | Pellegrini .....        | 204/129     |
| 4,219,443  | 8/1980  | Klinedinst et al. ..... | 252/425.3   |

Primary Examiner—John F. Niebling

Attorney, Agent, or Firm—Arthur S. Collins; Bruce E. Harang

## [57] ABSTRACT

A catalytic electrode has an electrically conductive substrate such as titanium or lead and is provided with a coating comprising a platinum-group metal catalyst finely dispersed in a matrix consisting of a semi-conducting polymer formed in situ on the substrate. The catalyst may be a platinum-group metal oxide such as iridium oxide formed in situ together with the semi-conducting polymer by a controlled heat treatment.

The semi-conducting polymer is preferably formed from polyacrylonitrile, polybenzimidazo-pyrrolone or an adamantane based polybenzoxazole.

5 Claims, No Drawings

**ELECTRODE COATING WITH  
PLATINUM-GROUP METAL CATALYST AND  
SEMI-CONDUCTING POLYMER**

**CROSS-REFERENCE TO RELATED  
APPLICATIONS**

This application is a continuation-in-part of copending application Ser. No. 282,182, filed May 21, 1981, now U.S. Pat. No. 4,402,996.

**FIELD OF THE INVENTION**

The present invention relates to dimensionally stable electrodes with a catalytic coating on an electroconductive substrate, and more particularly to their manufacture.

**BACKGROUND OF THE INVENTION**

Catalytic electrodes having a valve metal base and a catalytic coating comprising at least one platinum-group metal oxide are described for example in the following patents:

- U.K. Pat. No. 1,147,442
- U.K. Pat. No. 1,195,871
- U.K. Pat. No. 1,231,280
- U.K. Pat. No. 1,235,570
- U.S. Pat. No. 3,687,724

Dimensionally stable anodes of the type described in U.K. Pat. No. 1,195,871 are currently used for the electrolytic production of chlorine and provide a high anode life with reduced energy consumption.

However, when such anodes are used in metal electrowinning processes where oxygen is produced at the anode, they tend to undergo passivation and thus have a relatively short useful life. Passivation seems to be caused in this case by diffusion of oxygen through the coating resulting in build-up of an insulating oxide layer on the valve metal substrate and/or dissolution of ruthenium in the surrounding acid medium. In U.S. Pat. No. Re. 29,419, a coating is described which is especially intended as an anode for electrowinning. Finely divided ruthenium dioxide used as an electrocatalyst is applied together with an organic polymer to a substrate, followed by curing to produce a coating comprising the electrocatalyst dispersed in an inert polymer matrix. The organic polymer is intended in this case to serve as a binder, to provide mechanical support for the electrocatalyst to provide adhesion to and protection of the underlying substrate. According to the application intended, the amount of electrocatalyst used per part by weight of the polymer may generally vary within the range from 6:1 to 1:1, in order to provide the desired properties of such a coating. The conductive properties of such a composite coating will thus depend essentially on the amount of electrocatalyst dispersed in the inert polymer matrix, as well as its size and distribution throughout the matrix. The electrocatalyst must moreover be prepared in the form of extremely fine particles of less than 0.1 micron size, and then applied together with the organic polymer as uniformly as possible in order to be able to ensure the desired properties of the coating.

The state of the art relating to composite electrodes comprising conductive fillers dispersed in a polymer matrix may be further illustrated by U.S. Pat. Nos. 3,629,007, 3,751,301 and 4,118,294. The German patent application Offenlegungsschrift No. 2035918 further relates to an electrode for electrolytic purposes, which

comprises a metallic support coated with an organic semi-conductor consisting of a polymeric metal phthalocyanine. U.S. Pat. Nos. 3,792,732, 3,881,957 and 4,090,979 moreover relate to catalytic electrode materials comprising semi-conducting polymers formed on a refractory oxide and impregnated with metal catalysts.

The production of satisfactory catalytic coatings for dimensionally stable electrodes presents in fact many complex problems due to the severe technical and economic requirements of industrial electrolytic processes. These problems relate on one hand to the choice of suitable materials to provide adequate catalytic activity and conductivity, as well as being physically and electrochemically stable under the severe operating conditions of industrial electrolytic processes, such as high current density, corrosive media and products. Good electrocatalysts such as the platinum-group metal oxides are moreover very expensive so that they must generally be used in minimum amounts and combined with cheaper inert coating materials which, however, are generally catalytically inactive and electrically non-conductive (e.g.  $TiO_2$  and most organic polymers). On the other hand, many potentially interesting electrode materials may be unsuitable for the manufacture of satisfactory coatings which meet all requirement of industrial electrolytic processes. Thus, for example, various organic semi-conductors of potential interest as electrode materials, are relatively difficult to manufacture and moreover are difficult to process into satisfactory coatings.

It is an object of the present invention to provide an electrocatalytic coating comprising at least one platinum-group metal catalyst forming a uniform solid mixture with an insoluble semi-conducting polymer on an electroconductive substrate. Another object of the invention is to provide a simple process for the industrial manufacture of electrocatalytic coatings comprising at least one platinum-group metal catalyst and an insoluble semi-conducting polymer forming a uniform mixture on an electroconductive substrate.

Lead or lead alloy anodes are widely used for electrowinning metals from sulphate solutions but nevertheless exhibit various important limitations such as for example:

- (a) high anode potential
- (b) restricted anode current density and current efficiency
- (c) loss of anode materials with consequent contamination of the electrolyte and the electrowon metal product.

The use of alloyed lead may to a certain extent reduce the anode potential and improve the current efficiency, but the above limitations nevertheless remain as a whole.

**SUMMARY OF THE INVENTION**

The present invention provides an electrocatalytic coating comprising a platinum-group metal catalyst, more particularly a platinum-group metal oxide, which is finely dispersed in a semi-conducting, insoluble polymer matrix formed in situ on an electrically conductive substrate, whereby to form a catalytic electrode suitable for use in electrolytic process. The invention more particularly provides a process for manufacturing an electrocatalytic coating comprising at least one platinum-group metal catalyst and a polymer material applied to an electrically conductive substrate, as set forth in the

claims. This process comprises applying to a substrate a uniform liquid mixture including a predetermined amount of at least one platinum-group metal compound which can be thermally converted to said platinum-group metal catalyst, said liquid mixture further including at least one polymer which can be thermally converted to a semi-conducting insoluble polymer, said liquid mixture being successively applied in layers to the substrate and each layer being dried before the next layer is applied.

The process of the invention further comprises subjecting the resulting dried layers to heat treatment so as to form the platinum-group metal catalyst from said compound, together with said semi-conducting insoluble polymer and to thereby produce a coating consisting of a uniform solid mixture wherein the platinum-group electrocatalyst is finely dispersed in the semi-conducting insoluble polymer.

Platinum-group metals may be used as catalysts in any suitable form in the coatings of the invention, especially in the form of platinum-group metal oxides, which are particularly stable and may be simply produced according to the invention.

The substrate used in the invention may advantageously consist of an electrochemical valve metal such as titanium, in order to provide the well known advantages of valve metals as electrode substrates.

The uniform liquid mixture applied to the substrate according to the invention is preferably a homogeneous solution whereby to obtain a homogeneous mixture of the coating precursor materials dissolved in the form of molecules or ions. Emulsions may nevertheless be applied instead of homogeneous solutions if necessary e.g. in case the solvents used to respectively dissolve the organic and inorganic coating precursors may be non-miscible, among other reasons.

The solvents used in said liquid mixture will generally be any suitable conventional solvents such as e.g. dimethyl formamide (DMF) to dissolve polyacrylonitrile (PAN) or isopropyl alcohol (IPA) to dissolve  $\text{IrCl}_3$  or the like. Semiconducting insoluble polymers may be formed in coatings according to the invention by starting from various soluble polymers which can be thermally activated so as to undergo a structural change by extensive cross-linking and cyclization, whereby to form aromatic or heteroaromatic rings, so as to thus be able to form a substantially continuous planar semi-conducting polymer structure.

Polyacrylonitrile (PAN) was successfully applied in solution to produce a coating according to the invention. However, some other polymers which may be suitable are: polyacrylamide or other derivatives of polyacrylic acid. Soluble aromatic polymers may also be used in the invention, such as for example: aromatic polyamides, aromatic polyesters, polysulfones, aromatic polysulphides, epoxy, phenoxy, or alkyd resins containing aromatic building blocks, polyphenylene or polyphenylene oxides. Heteroaromatic polymers may further be suitable for the invention, such as for example polyvinyl pyridine, polyvinylpyrrolidone, or polytetrahydrofuran. Prepolymers may likewise be suitable which are convertible to heteroaromatic polymers, such as for example, polybenzoxazoles or polybenzimidazopyrrolones. Polymers containing adamantine may likewise be suitable (especially the above prepolymers, containing adamantine units). Polybenzimidazopyrrolone (pyrrole) and adamantine based polybenzoxazole (PBO) were applied in solution (in

5 N-methyl pyrrolidone) to produce coatings according to the invention.

A coating may be produced according to the invention by applying any suitable number of layers of solution which is necessary to provide the desired thickness and surface loading while ensuring satisfactory adherence of the coating. Each dried layer of solution provides a uniform coprecipitated intimate mixture of a very finely divided catalyst precursor and the organic polymer matrix precursor.

10 The heat treatment of this coprecipitate is then advantageously effected in air in at least two stages at different temperatures, preferably with a reduced temperature stage in the range up to about 300° C., before applying the next layer of solution and, after applying the last layer, an elevated-temperature stage at about 400° C., but at most up to 500° C. The temperature range, duration, and ambient atmosphere of heat treatment should be controlled so as to be able to ensure extensive cross-linking and cyclization of the organic polymer precursor by thermal activation, so as to convert it into a substantially continuous semi-conducting, insoluble, polymeric network structure, while substantially preventing thermal decomposition of the organic polymer structure or carbonization of the organic polymer. These conditions of heat treatment must at the same time be selected so as to also allow conversion of the coprecipitated catalyst precursor compound into a finely divided catalyst, uniformly dispersed and completely integrated in said semi-conducting polymer network structure forming a substantially continuous matrix. One heat treatment stage in air may be carried out for example in a reduced temperature range between 250° C. and 300° C., while a subsequent stage may be carried out in air in a higher range between 300° C. and 400° C., or somewhat higher, e.g. 500° C. or even up to 600° C. in some instances. Moreover, the reduced temperature heat treatment stage in air may if necessary be followed by a heat treatment stage in a non-oxidative or inert atmosphere such as nitrogen, possibly to higher temperatures up to 800° C., for a duration for example between 15 minutes and 6 hours. The duration of heat treatment in air may vary from 5 minutes to about 2 hours according to the nature of the organic polymer. It may be noted that heat treatment in air according to the invention can provide platinum-group metal oxides at relatively low temperatures up to 400° C., while at the same time providing a semiconducting polymer matrix. On the other hand, conventional coatings comprising platinum-group metal oxides alone, or in combination with other inorganic oxides generally require higher temperatures. Semiconducting polymeric coatings were produced by applying several layers of PAN in solution in DMF to conductive substrates, drying, and heat treating, as described above and in the examples given further on. It was experimentally established that the coatings thus produced from PAN became semiconductive after undergoing a heat treatment stage at 300° C. in air.

15 The invention allows substantial advantages to be achieved by means of a very simple combination of steps which can be carried out reproducibly at low cost and only require relatively simple equipment for the preparation, application and drying of exactly predetermined liquid compositions, and for controlled heat treatment.

20 Thus, for example, the invention may provide the following advantages:

(i) A semi-conducting, insoluble, stable polymer matrix is formed directly in situ on the substrate surface, by controlled application of a predetermined polymer containing liquid composition, followed by controlled heat treatment.

(ii) The catalyst simultaneously formed in situ is uniformly distributed throughout the semi-conducting polymer matrix so as to provide a consolidated coating of uniform composition.

(iii) This uniform distribution thus allows the catalyst to be used as effectively as possible, i.e. a minimum amount of platinum-group metal catalyst needs to be incorporated in the coating in order to provide adequate catalytic properties.

(iv) On the other hand, the semi-conducting polymer matrix itself provides adequate current conduction and uniform current distribution throughout the coating, thereby allowing it to support high current densities.

(v) The semi-conducting insoluble polymer matrix is moreover relatively stable and resistant to both physical and electrochemical attack, and thus may serve as a semi-conducting protective binder for the catalyst, while at the same time protecting the underlying substrate and promoting adherence of the coating to the substrate.

(vi) The above advantages may more particularly provide corrosion resistant dimensionally stable electrodes of the invention with stable electrochemical performance and a long useful life under severe operating conditions.

Electrodes coated according to the invention may be used advantageously as anodes at which oxygen is evolved, in order to more particularly provide protection of the catalyst as well as the underlying substrate. They may thus be used more particularly as anodes in electrowinning processes. The electrodes of the invention may moreover be suitable as anodes for water electrolysis. Coated electrodes of the invention may also meet the requirements of anodes for the production of chlorine or chlorate. In this case the anode coating may comprise for example a ruthenium dioxide catalyst, with additions of oxides of Sn, Pd, and/or Pb, e.g. in order to increase the oxygen over-potential. Moreover, electrodes coated according to the invention may also be usefully applied as cathodes, e.g. as cathodes at which hydrogen is generated, in chloralkali processes, water electrolysis, or other electrolytic processes.

It may be noted that platinum-group metal catalysts may be used in the metallic state in the coatings of the invention, by precipitation of any suitable soluble platinum-group metal compound when drying the applied liquid mixture, and subsequent thermal conversion of said compound to the platinum-group metal in the metallic state.

It may be noted that other materials may be uniformly incorporated in the coating according to the invention in generally the same manner as the platinum-group metal catalysts. Such materials may serve to provide given properties, e.g. to further improve conductivity and/or catalytic activity of the coating, to inhibit undesirable side-reactions (e.g. to raise the oxygen over-potential on anodes for chlorine production), to improve physical or chemical stability of the coating. The liquid mixture applied to the substrate according to the invention may moreover contain various additives to enhance the formation of a satisfactory semi-conducting polymer matrix e.g. cross-linking agents.

The invention also provides a catalytic electrode comprising a body of lead or lead alloy with an electrocatalytic coating having a catalyst finely dispersed in an insoluble, semi-conducting polymer matrix formed in situ on the surface of said body.

The invention further provides a method of coating and catalytically activating an electrode of lead or lead alloy, as set forth in the claims.

A finely dispersed platinum group metal catalyst may be advantageously formed from any suitable inorganic compound in the coating produced according to the invention.

The catalytically activated, coated lead or lead alloy electrodes according to the invention are particularly

suitable for use as oxygen-evolving anodes in acid electrolytes, e.g. in metal electrowinning processes, whereby to provide improved electrolytic performance with respect to lead or lead alloy anodes currently used for this purpose. The electrodes according to the invention may also be used as anodes for other applications. They may also be useful as cathodes for certain electrolytic processes.

Such an electrode comprising a body of lead or lead alloy with a catalytic coating according to the invention more particularly provides the following advantages:

1. It can be operated as an anode for oxygen evolution with a half-cell potential which is significantly lower than that of conventional lead or lead alloy anodes currently used for electrowinning metals.

2. The anode current density may be increased while maintaining a cell-voltage equal to or lower than that generally applied in conventional metal electrowinning cells, so that the energy costs may be reduced accordingly.

3. The electrocatalytic coating operates at a reduced anode potential and at the same time effectively protects the underlying lead or lead alloy base which now essentially functions as a conductive support and is electrochemically inactive at the reduced anode potential, whereby the loss of anode materials during operation may be significantly reduced.

4. Conventional lead or lead alloy anodes may be readily converted into an anode by coating according to the invention. It thus becomes possible to directly retrofit industrial cells for electrowinning metals in a particularly simple and inexpensive manner so as to obtain the advantages of the invention. This can be rapidly done by removing the existing anodes, coating them, replacing them in the cell for operation, and recoating whenever necessary.

5. Other catalysts suitable for oxygen evolution such as manganese dioxide for example may likewise be applied in a particularly simple manner in accordance with the invention.

55 The invention is illustrated in the following examples with reference to experimental data in the accompanying tables.

These tables indicate the following:

The reference of each coated electrode sample  
The number of layers and type of each solution applied to the coating substrate

The initial loading of the main components applied in solution per unit area of the substrate surface

The conditions of the heat treatment of said components for producing a coating

The anode current density under which each electrode sample was tested as an oxygen-evolving anode in an electrolysis cell containing 350 cc of

150 g/l H<sub>2</sub>SO<sub>4</sub> aq. and two graphite cathodes of 100×20 mm projected area respectively disposed at a distance of 25 mm from each face of the anode. The initial anode potential of each electrode sample with respect to a normal hydrogen electrode (NHE), as well as the final potential at the end of the test period (unless the anode has failed due to a steep rise of its potential)

Finally the duration of each test period in hours, the time being marked with an asterisk if the anode is 10 still operating or underlined if the electrode has failed.

### EXAMPLE 1

Several titanium plates (100×20×1 mm) were pre-treated by sand-blasting followed by an etching treatment in 10% oxalic acid at about 85° C. for 6 hours, whereby to form a microrough surface. The pretreated titanium plates were then coated to produce the electrode samples D92, C92, B08, F31, F58, D36, D72, D77 which are shown in Table 1 below.

Homogeneous solutions for producing a coating comprising iridium oxide and a semi-conducting polymer were prepared by mixing a solution of polyacrylonitrile (PAN) in dimethyl formamide (DMF) with an acid solution of IrCl<sub>3</sub>aq. in isopropyl alcohol (IPA).

Three solutions prepared in this manner respectively contained the following amounts of iridium and PAN per gram of solution:

|      |            |             |
|------|------------|-------------|
| P15a | 7 mg Ir    | 18.6 mg PAN |
| P15  | 14.7 mg Ir | 16.4 mg PAN |
| P15c | 14.7 mg Ir | 24.3 mg PAN |

Each of these solutions was successively applied with a brush in several layers to one of said titanium plates so as to cover the entire plate surface.

The second column in Table 1 shows for each electrode sample the corresponding number of layers and the type of solution applied.

The third column in Table 1 indicates the corresponding initial loadings of Ir and PAN in grams per square meter of the titanium plate surface.

After applying each layer of solution to the titanium plate, it was subjected to drying in an oven at 100° C. for 5 minutes, and then subjected to a first heat treatment at 250° C. for 10 minutes in a stationary air atmosphere, as indicated under I in Table 1.

After applying the last layer, drying and heating as described, a second heat treatment was carried out at 300° C. for a period of 7 or 30 minutes in stationary air or in an air flow of 60 l/h as indicated under II in Table 1. This was followed by a third heat treatment at 400° C. for 7.5; 20; or 15 minutes, as indicated under III in Table 1.

The resulting coated electrode samples were then tested as an oxygen-evolving anode in an electrolysis

cell containing concentrated sulphuric acid, as previously mentioned.

The anode potential of the respective electrode samples was monitored during each electrolytic test. As already mentioned, Table 1 indicates the initial anode potential (vs. NHE), for each test of a given electrode sample at the indicated current density, while the final anode potential at the end of each test is also indicated, unless the anode has failed as a result of a steep substantial rise of its potential.

The following may be noted with regard to the electrolytic test results shown in Table 1:

The electrode sample D92 with a catalytic coating having a relatively low loading of iridium oxide corresponding to 1.7 g Ir/m<sup>2</sup> and a much higher PAN loading of 4.5 g/m<sup>2</sup>, operated at 500 A/m<sup>2</sup> for 1350 hours, with an initial potential of 1.60 V/NHE, and is still operating.

The electrode sample D72 with a higher loading of 3 gIr/m<sup>2</sup> and a lower loading of 3.6 g PAN/m<sup>2</sup> has a slightly higher anode potential (1.65 V/NHE) at 500 A/m<sup>2</sup> and failed after 1690 hours.

The electrode samples C92, B08, F31, F58, D36 and D77 were first tested at 500 A/m<sup>2</sup> and showed only a slight increase in potential with no notable sign of deterioration. The current density was then increased to 2500 A/m<sup>2</sup>. Sample F31 is still operating at 2500 A/m<sup>2</sup> after 820 hours with no considerable increase in potential. The performance of D72 and D77 is lower than expected in view of the loading of both components and the heat treatment. One possible explanation is the low number of layers applied (corresponding to very thick layers). The premature failure of F58 may be caused by the too prolonged final heat treatment under these specific preparation conditions.

For reference, the electrode samples C94, C95 and G24 in Table 1 were prepared in substantially the same manner as in Example 1, but without including PAN in the solutions applied to the titanium plate. The solution WP15b applied to produce these samples comprised IrCl<sub>3</sub>aq. dissolved in IPA as before, and was further diluted with DMF to provide the same iridium concentration of 14.7 mgIr/g, as in the case of the solutions P15 and P15c. Electrode samples C94 and C95 (prepared without PAN) which were coated and heat treated in three stages failed rapidly at 2500 A/m<sup>2</sup>, whereas the other coatings in Table 1 had a significant lifetime at this current density. The electrode sample G24 was prepared by heat treatment under conditions suitable for obtaining a good iridium oxide coating on a titanium substrate. 10 layers were applied and after drying each layer at 100° C. for 5 minutes, the sample was heat treated at 480° C. for 7 minutes in an air flow of 60 l/h. This sample is still running at 2500 A/m<sup>2</sup> after 350 hours. However, the potential of 2.33 V is higher than the corresponding values of other electrode samples in Table 1 such as F31.

TABLE 1

| REF            | SOLUTION APPLIED |                                           | HEAT TREATMENT        |                        |                         | TEST CONDITIONS                           |                          |             |
|----------------|------------------|-------------------------------------------|-----------------------|------------------------|-------------------------|-------------------------------------------|--------------------------|-------------|
|                | LAYERS<br>SOLN.  | INITIAL<br>LOADING<br>(g/m <sup>2</sup> ) | I<br>(°C-min)<br>atm. | II<br>(°C-min)<br>atm. | III<br>(°C-min)<br>atm. | CURRENT<br>DENSITY<br>(A/m <sup>2</sup> ) | ANODE<br>POT.<br>(V/NHE) | TIME<br>(h) |
| D 92<br>(P15a) | 8                | 1.7 Ir + 4.5 PAN                          | 250-10<br>stat. air   | 300-7<br>stat. air     | 400-20<br>air 60 l/h    | 500                                       | 1.6-2.1                  | 1350*       |
|                | 5                | 2.0 Ir + 2.3 PAN                          | 250-10<br>stat. air   | 300-30<br>air 60 l/h   | 400-7.5<br>air 90 l/h   | 500                                       | 1.67-1.68                | 227         |
| C 92<br>(P15)  | 5                | 2.0 Ir + 2.3 PAN                          | 250-10<br>stat. air   | 300-30<br>air 60 l/h   | 400-7.5<br>air 90 l/h   | 2500                                      | 1.70-fail                | 767         |
|                | 5                | 2.0 Ir + 2.3 PAN                          | 250-10<br>stat. air   | 300-30<br>air 60 l/h   | 400-7.5<br>air 90 l/h   | 500                                       | 1.58-1.69                | 577         |
| B 08<br>(P15)  |                  |                                           |                       |                        |                         | 2500                                      | 1.73-fail                | 737         |

TABLE 1-continued

| REF  | LAYERS<br>SOLN. | SOLUTION APPLIED | HEAT TREATMENT                            |                       |                        | TEST CONDITIONS         |                                           |                          |
|------|-----------------|------------------|-------------------------------------------|-----------------------|------------------------|-------------------------|-------------------------------------------|--------------------------|
|      |                 |                  | INITIAL<br>LOADING<br>(g/m <sup>2</sup> ) | I<br>(°C-min)<br>atm. | II<br>(°C-min)<br>atm. | III<br>(°C-min)<br>atm. | CURRENT<br>DENSITY<br>(A/m <sup>2</sup> ) | ANODE<br>POT.<br>(V/NHE) |
| F 31 | 6<br>(P15)      | 1.9 Ir + 2.1 PAN | 250-10                                    | 300-30                | 400-15                 | 500                     | 1.67-1.69                                 | 130                      |
|      |                 |                  |                                           | stat. air             | air 60 l/h             | air 90 l/h              | 2500                                      | 1.74-1.90                |
| F 58 | 6<br>(P15)      | 2.2 Ir + 2.5 PAN | 250-10                                    | 300-30                | 400-20                 | 500                     | 1.65-1.68                                 | 120                      |
|      |                 |                  |                                           | stat. air             | air 60 l/h             | air 60 l/h              | 2500                                      | 1.80-fail                |
| D 36 | 5<br>(P15)      | 3.2 Ir + 3.6 PAN | 250-10                                    | 300-30                | 400-7.5                | 500                     | 1.63-1.67                                 | 350                      |
|      |                 |                  |                                           | stat. air             | air 60 l/h             | air 90 l/h              | 2500                                      | 1.73-fail                |
| D 72 | 3<br>(P15c)     | 3 Ir + 5.1 PAN   | 250-10                                    | 300-30                | 400-7.5                | 500                     | 1.64-fail                                 | 1690                     |
|      |                 |                  |                                           | stat. air             | air 60 l/h             | air 90 l/h              |                                           |                          |
| D 77 | 3<br>(P15c)     | 2.2 Ir + 3.6 PAN | 250-10                                    | 300-30                | 400-7.5                | 500                     | 1.68-1.72                                 | 150                      |
|      |                 |                  |                                           | stat. air             | air 60 l/h             | air 90 l/h              | 2500                                      | 1.71-fail                |
| C 94 | 5<br>(WP15b)    | 2 Ir             | 250-10                                    | 300-30                | 400-7.5                | 500                     | 1.70-1.93                                 | 87                       |
|      |                 |                  |                                           | stat. air             | air 60 l/h             | air 90 l/h              | 2500                                      | 2.10-fail                |
| C 95 | 5<br>(WP15b)    | 2 Ir             | 250-10                                    | 300-30                | 400-7.5                | 500                     | 1.71-                                     | 87                       |
|      |                 |                  |                                           | stat. air             | air 60 l/h             | air 90 l/h              | 2500                                      | 1.83-fail                |
| G 24 | 10<br>(WP15b)   | 2 Ir             | —                                         | —                     | 10 × 480-7             | 500                     | 1.86-1.87                                 | 300                      |
|      |                 |                  |                                           |                       | air 60 l/h             | 2500                    | 1.85-2.33                                 | 350*                     |

## EXAMPLE 2

The electrode samples shown in Table 2 were prepared in the manner described in Example 1, by successively applying to a similar pretreated titanium plate layers of a solution containing both  $\text{IrCl}_3$  and PAN, followed by drying and heat treatment. 25

Table 2, which is drawn up in the same manner as Table 1, shows that various modifications were made in the heat treatments to which the electrode samples were 30

This table shows again the predominant role of the heat treatment.

Electrode sample F71 which was subjected to the heat treatments I at  $250^\circ\text{C}$ . and II at  $300^\circ\text{C}$ . (for a longer period of 60 minutes), but not to a third heat treatment III at a higher temperature, failed after 5 hours at a reduced current density of only  $250\text{ A/m}^2$ .

The final heat treatment at  $450^\circ\text{C}$ . with steps I and II also shows a deterioration.

TABLE 2

| REF  | LAYERS<br>SOLN. | SOLUTION APPLIED  | HEAT TREATMENT                            |                       |                        | TEST CONDITIONS         |                                           |                          |
|------|-----------------|-------------------|-------------------------------------------|-----------------------|------------------------|-------------------------|-------------------------------------------|--------------------------|
|      |                 |                   | INITIAL<br>LOADING<br>(g/m <sup>2</sup> ) | I<br>(°C-min)<br>atm. | II<br>(°C-min)<br>atm. | III<br>(°C-min)<br>atm. | CURRENT<br>DENSITY<br>(A/m <sup>2</sup> ) | ANODE<br>POT.<br>(V/NHE) |
| F 78 | 7<br>(P15)      | 1.8 Ir + 2 PAN    | 250-10                                    | —                     | 400-15                 | 500                     | 1.64-1.71                                 | 150                      |
|      |                 |                   |                                           | stat. air             | air 60 l/h             | 2500                    | 1.75-1.92                                 | 750*                     |
| F 83 | 7<br>(P15)      | 1.8 Ir + 2 PAN    | 250-10                                    | —                     | 430-15                 | 500                     | 1.64-1.72                                 | 150                      |
|      |                 |                   |                                           | stat. air             | air 60 l/h             | 2500                    | 1.82-1.96                                 | 700*                     |
| F 52 | 4<br>(P15a)     | 0.8 Ir + 2.1 PAN  | —                                         | 300-7                 | 400-10                 | 500                     | 1.60-2.00                                 | 1000*                    |
|      |                 |                   |                                           | stat. air             | air 60 l/h             |                         |                                           |                          |
| C 53 | 4<br>(P15a)     | 0.85 Ir + 2.3 PAN | —                                         | 300-7                 | 400-10                 | 500                     | 1.85-fail                                 | 1526                     |
|      |                 |                   |                                           | stat. air             | air 60 l/h             |                         |                                           |                          |
| C 55 | 4<br>(P15a)     | 0.85 Ir + 2.3 PAN | —                                         | 300-7                 | 450-15                 | 500                     | 1.7-fail                                  | 1165                     |
|      |                 |                   |                                           | stat. air             | air 60 l/h             |                         |                                           |                          |
| F 99 | 4<br>(P15a)     | 0.6 Ir + 1.6 PAN  | 250-10                                    | —                     | 350-10                 | 500                     | 2.3-fail                                  | 0.03                     |
|      |                 |                   |                                           | stat. air             | air 60 l/h             |                         |                                           |                          |
| F 75 | 6<br>(P15)      | 2.4 Ir + 2.7 PAN  | —                                         | 300-30                | 415-7.5                | 500                     | 1.64-2.05                                 | 207                      |
|      |                 |                   |                                           | air 60 l/h            | air 60 l/h             | 2500                    | 2.04-fail                                 | 13                       |
| F 71 | 6<br>(P15)      | 2.4 Ir + 2.7 PAN  | 250-10                                    | 300-60                | —                      | 250                     | 1.64-fail                                 | 5                        |
|      |                 |                   |                                           | stat. air             | air 60 l/h             |                         |                                           |                          |

subjected in this case.

Thus, as it may be seen from Table 2:

The second heat treatment II at  $300^\circ\text{C}$ . previously described was omitted in the case of samples F78 and F83;

The first heat treatment I at  $250^\circ\text{C}$ . was omitted in the case of samples F52, C53 and C55

The last heat treatment III was omitted in the case of sample F71

The highest heat treatment temperature of sample 65 F83 was raised to  $430^\circ\text{C}$ . and of sample C55 to  $450^\circ\text{C}$ .

## EXAMPLE 3

The electrode samples shown in Table 3 were prepared as described in Example 1, although the last heat treatment III was effected in a nitrogen atmosphere at a flow rate of 6 l/h, at higher temperature between  $500^\circ\text{C}$ . and  $650^\circ\text{C}$ ., and were heated up to these temperatures at different controlled heating rates, which are respectively indicated under III in Table 3.

Moreover, the intermediate heat treatment II was omitted in the case of the electrode samples F82 and G63. The best results were obtained for F82 with a rather fast heating rate of  $300^\circ\text{C./h}$  without step II.

TABLE 3

| REF  | SOLUTION APPLIED |                                           | HEAT TREATMENT         |                         |                                              | TEST CONDITIONS                           |                          |             |
|------|------------------|-------------------------------------------|------------------------|-------------------------|----------------------------------------------|-------------------------------------------|--------------------------|-------------|
|      | LAYERS<br>REF    | INITIAL<br>LOADING<br>(g/m <sup>2</sup> ) | I<br>(°C.-min)<br>atm. | II<br>(°C.-min)<br>atm. | III<br>(°C.-min)<br>atm.                     | CURRENT<br>DENSITY<br>(A/m <sup>2</sup> ) | ANODE<br>POT.<br>(V/NHE) | TIME<br>(h) |
| F 82 | 7<br>(P15)       | 1.8 Ir + 2.0 PAN                          | 250-10<br>Stat. air    | —                       | 500-30<br>N <sub>2</sub> -6 l/h<br>300° C./h | 500                                       | 1.71-1.75                | 750*        |
| F 68 | 6<br>(P15)       | 2.2 Ir + 2.5 PAN                          | —                      | 300-30<br>air 60 l/h    | 500-30<br>N <sub>2</sub> -6 l/h<br>200° C./h | 500                                       | 1.76-fail                | 12-15       |
| G 63 | 6<br>(P15)       | 2 Ir + 2.2 PAN                            | 250-10<br>Stat. air    | —                       | 550-30<br>N <sub>2</sub> -6 l/h<br>350° C./h | 250                                       | 1.59-fail                | 40          |
| D 94 | 8<br>(P15a)      | 1.7 Ir + 4.5 PAN                          | 250-10<br>Stat. air    | 300-7<br>Stat. air      | 650-30<br>N <sub>2</sub> -6 l/h<br>200° C./h | 500                                       | 1.60-fail                | 0.3         |

## EXAMPLE 4

The electrode samples shown in Table 4 were prepared in the manner described in Example 1, Ru or Pt being included besides Ir and PAN, and Ir being the minor component. Two solutions were prepared with the following amounts of solutes per gram of solution, the solvents being IPA and DMF as before:

|     |           |            |             |
|-----|-----------|------------|-------------|
| P58 | 5 mg Ir   | 6 mg Ru    | 10 mg PAN   |
| P59 | 4.4 mg Ir | 10.3 mg Pt | 16.4 mg PAN |

In addition, the number of layers of P58 applied was respectively increased to 9 (for G17), 12 (F84) and 14 (for F92). As may be seen from the loadings shown in Table 5, the coatings contained here much less iridium than before, while the ruthenium content amounted to 75% of the platinum-group metal loading.

A major part of the iridium may thus be replaced by ruthenium which has a much lower cost.

Table 4 shows good performance for the electrode sample F84 and F92 which are still operating. The potential of electrode samples G51 and G52 containing Pt is somewhat higher after 200 hours of operation.

contained, in addition to IrCl<sub>3</sub>aq. the following starting polymer (instead of PAN, as before). Polybenzimidazopyrrolone (pyrrole) or adamantane based polybenzoxazole (PBO). The solutions used in this case had the following compositions:

|     |                   |                         |
|-----|-------------------|-------------------------|
| PP5 | 7.1 mg Ir/g soln. | 18.8 mg Pyrrole/g soln. |
| PP6 | 7.0 mg Ir/g soln. | 18.6 mg PBO/g soln.     |

The solvent was NMP (N-methyl pyrrolidone) in this case.

As appears from the results shown in Table 5: The electrode sample D91 with pyrrole as the starting polymer failed after 354 hours at 500 A/m<sup>2</sup>. On the other hand, the electrode sample D96 (also with pyrrole), which was heat treated in nitrogen at 650° C., failed after 15 hours. Moreover, the electrode sample F1 which comprised PBO as the starting polymer and was heat treated in the same way as the sample D96, failed after 125 hours at 500 A/m<sup>2</sup>.

The electrode sample F3 operated for 1350 hours at 500 A/m<sup>2</sup> without any change in its initial potential of 1.7 V/NHE.

TABLE 4

| REF  | SOLUTION APPLIED |                                           | HEAT TREATMENT         |                         |                          | TEST CONDITIONS                           |                          |             |
|------|------------------|-------------------------------------------|------------------------|-------------------------|--------------------------|-------------------------------------------|--------------------------|-------------|
|      | LAYERS<br>REF    | INITIAL<br>LOADING<br>(g/m <sup>2</sup> ) | I<br>(°C.-min)<br>atm. | II<br>(°C.-min)<br>atm. | III<br>(°C.-min)<br>atm. | CURRENT<br>DENSITY<br>(A/m <sup>2</sup> ) | ANODE<br>POT.<br>(V/NHE) | TIME<br>(h) |
| F 84 | 12<br>(P58)      | 0.5 Ir + 1.5 Ru +<br>2.50 PAN             | 250-10<br>stat. air    | 300-30<br>air 60 l/h    | 400-10<br>air 60 l/h     | 500                                       | 1.64-1.68                | 600*        |
| F 92 | 14<br>(P58)      | 0.5 Ir + 1.5 Ru +<br>2.50 PAN             | 250-10<br>stat. air    | 300-30<br>air 60 l/h    | 415-10<br>air 60 l/h     | 500                                       | 1.71-1.67                | 150*        |
| G 17 | 9                | 0.3 Ir + 0.9 Ru +<br>1.6 PAN              | —                      | —                       | 400-2.5<br>air 60 l/h    | 500                                       | 1.65-fail                | 430         |
| G 51 | 7<br>(P59)       | 1 Ir + 2.2 Pt +<br>3.6 PAN                | 250-10<br>Stat. air    | 300-10<br>air 60 l/h    | 430-15<br>air 60 l/h     | 500                                       | 1.77-1.80                | 200*        |
| G 52 | 7<br>(P59)       | 1 Ir + 2.2 Pt +<br>3.6 PAN                | 250-10<br>Stat. air    | 300-10<br>air 60 l/h    | 400-15<br>air 60 l/h     | 500                                       | 1.77-1.87                | 200*        |

## EXAMPLE 5

The electrode samples shown in Table 5 were prepared in the manner described in Example 1, but the homogeneous solutions applied in this case respectively

The heat treatment of samples D91 and F3 at 400° C. in air flow provides better results than the heat treatments of the corresponding samples D96 and F1 at 650° C. in nitrogen.

TABLE 5

| REF  | SOLUTION APPLIED |                                           | HEAT TREATMENT         |                         |                          | TEST CONDITIONS                           |                          |             |
|------|------------------|-------------------------------------------|------------------------|-------------------------|--------------------------|-------------------------------------------|--------------------------|-------------|
|      | LAYERS<br>REF    | INITIAL<br>LOADING<br>(g/m <sup>2</sup> ) | I<br>(°C.-min)<br>atm. | II<br>(°C.-min)<br>atm. | III<br>(°C.-min)<br>atm. | CURRENT<br>DENSITY<br>(A/m <sup>2</sup> ) | ANODE<br>POT.<br>(V/NHE) | TIME<br>(h) |
| D 91 | 8                | 1.7 Ir + 4.5 pyrrole                      | 250-10                 | 300-120                 | 400-20                   | 500                                       | 1.6-fail                 | 354         |

TABLE 5-continued

| REF  | SOLUTION APPLIED |       | HEAT TREATMENT                            |                        |                         | TEST CONDITIONS                    |                                           |                          |             |
|------|------------------|-------|-------------------------------------------|------------------------|-------------------------|------------------------------------|-------------------------------------------|--------------------------|-------------|
|      | LAYERS<br>REF    | SOLN. | INITIAL<br>LOADING<br>(g/m <sup>2</sup> ) | I<br>(°C.-min)<br>atm. | II<br>(°C.-min)<br>atm. | III<br>(°C.-min)<br>atm.           | CURRENT<br>DENSITY<br>(A/m <sup>2</sup> ) | ANODE<br>POT.<br>(V/NHE) | TIME<br>(h) |
| D 96 | (PP5)            | 8     | 1.7 Ir + 4.5 pyrrole                      | stat. air              | stat. air               | air 60 l/h                         | 500                                       | 1.6-fail                 | 15          |
|      |                  |       |                                           | 250-10                 | 300-120                 | 650-30                             |                                           |                          |             |
| F 3  | (PP5)            | 8     | 1.7 Ir + 4.5 PBO                          | stat. air              | stat. air               | N <sub>2</sub> -6 l/h<br>200° C./h | 500                                       | 1.7-1.7                  | 1350*       |
|      |                  |       |                                           | 250-10                 | 300-120                 | 400-20                             |                                           |                          |             |
| F 1  | (PP6)            | 8     | 1.7 Ir + 4.5 PBO                          | stat. air              | stat. air               | air 60 l/h                         | 500                                       | 1.7-fail                 | 125         |
|      |                  |       |                                           | 250-10                 | 300-120                 | 650-30                             |                                           |                          |             |
|      | (PP6)            |       |                                           | stat. air              | stat. air               | N <sub>2</sub> -6 l/h<br>200° C./h |                                           |                          |             |

## EXAMPLE 6

A solution (P63) containing poly-p-phenylene and IrCl<sub>3</sub>.aq. in dimethylformamide (DMF) was prepared with respective PPP and Ir concentrations of 36 and 8.2 mg/g solution.

A lead sheet was sandblasted and degreased prior to its coating with the above mentioned solution.

In one case, 8 layers were applied to the sample which was heat treated at 300° C. for 7.5 minutes after each layer. A final-postbaking was carried out under the same conditions. The respective Ir loading, after 8 layers, amounted to 1.1 g/m<sup>2</sup>. The resulting electrode was tested in 150 gpl H<sub>2</sub>SO<sub>4</sub> at 5000 A/m<sup>2</sup> as an oxygen evolving anode. It had a life time of 310 h under these conditions. The respective potential amounted to 2.15 V vs. NHE after 300 h of operation. The electrode was considered to have failed when the onset of lead corrosion was detected in this accelerated test.

Another sample was coated with the same starting solution, but the heat treatment, after each layer, prolonged to 10 minutes. No postbaking was carried out in this case. The electrode was tested at 1000 A/m<sup>2</sup> in 160 gpl H<sub>2</sub>SO<sub>4</sub> with an increase in its initial potential from 2.03 to 2.15 V vs. NHE after 1000 h of operation. The respective life time amounted to 1200 h.

Pb and Pb-Ag (0.5% Ag) anodes were tested for comparison. Both uncoated samples were tested at 1000 A/m<sup>2</sup>. In the case of Pb, the initial electrode potential increased from 2.92 V vs NHE to 5.63 V vs. NHE after 2 h of operation. In the case of Pb-Ag, the initial potential amounted to 2.23 V vs. NHE increasing to 4.72 V vs. NHE after 720 h of operation.

All electrode potentials are not corrected for the Ir-drop.

## EXAMPLE 7

The starting solution, described in Example 6 as well as the pretreatment, were applied to another Pb sheet.

In this case, however, only 4 layers were applied to give an Ir loading of 0.5 g/m<sup>2</sup>. The sample was heat treated at 310° C., under an airflow, for 10 minutes after each layer. After the last layer, an additional heat treatment was carried out for 30 minutes under identical conditions. The resulting anode was tested at 1000 A/m<sup>2</sup> and exhibited a potential of 2.11 vs. NHE after 1850 h of operation in 150 gpl H<sub>2</sub>SO<sub>4</sub>.

## EXAMPLE 8

A solution (P15e) containing polyacrylonitrile (PAN) and IrCl<sub>3</sub>.aq. in DMF was prepared with the respective concentrations of 17.9 mg and 9.6 mg/g solution for PAN and Ir.

A Pb-Ag (0.5% Ag) sample was sandblasted and degreased. Four layers of the above-mentioned solution were applied and heat treated at 320° C. for 10 minutes after each layer. An additional heat treatment was carried out for 1 h under the same conditions. The anode was tested at 1000 A/m<sup>2</sup> in 150 gpl H<sub>2</sub>SO<sub>4</sub> showing a potential of 1.99 V vs. NHE after 600 h of operation. The corresponding value of an uncoated Pb-Ag anode amounted to 2.34 V vs. NHE under the same conditions.

## EXAMPLE 9

The starting solution, described in Example 8, was applied to a lead sheet in 4 layers, dried and heat treated at 305° C. for 15 minutes after each layer.

The anode was tested at 500 A/m<sup>2</sup> in 150 gpl H<sub>2</sub>SO<sub>4</sub> and exhibited a potential of 1.89 V vs NHE after 1000 h of operation.

We claim:

1. A method of manufacturing an electrode with a body of lead or a lead alloy and an electrocatalytic, protective coating comprising at least one platinum group catalyst, characterized by the steps of
  - (a) applying to the surface of said electrode body of lead or lead alloy a solution containing at least one soluble organic polymer compound and one compound of a platinum group metal, which can be thermally converted respectively to a semi-conducting, insoluble polymer and to a platinum group catalyst;
  - (b) drying the applied solution and effecting controlled heat treatment at a temperature below the melting point of said electrode body of lead or lead alloy, so as to thermally convert said compounds into an electrocatalytic protective coating comprising said platinum group catalyst finely dispersed in a continuous matrix of said semi-conducting, insoluble polymer formed in situ and adhering to said surface of the electrode body of lead or lead alloy; and
  - (c) repeating said step (a) plus step (b) sequence until an electrocatalytic protective coating of the desired thickness is attained.
2. A method of catalytically activating an electrode body of lead or a lead alloy by means of a platinum group catalyst, characterized by the steps of
  - (a) applying to the surface of said electrode body of lead or lead alloy a solution containing at least one soluble organic polymer compound and one compound of a platinum group metal, which can be thermally converted respectively to a semi-conducting insoluble polymer and to a platinum group catalyst;

(b) drying the applied solution and effecting controlled heat treatment at a temperature below the melting point of said electrode body of lead or lead alloy, so as to thermally convert said compounds into an electrocatalytically active, protective coating comprising said platinum group catalyst finely dispersed in a continuous matrix of said semi-conducting insoluble polymer formed in situ and ad-

hering to said surface of the electrode body of lead or lead alloy.

3. The method of claim 1 or 2 wherein said organic polymer compound which is dissolved in the solution applied in step (a), is selected from the group consisting of polyacrylonitrile and poly-p-phenylene.

4. The method of claim 3 wherein said heat treatment in step (b) is carried out in the presence of air.

5. The method of claim 1 or 2 wherein said heat treatment in step (b) is carried out in the presence of air.

\* \* \* \* \*

15

20

25

30

35

40

45

50

55

60

65